

# United States Patent

[11] 3,615,430

[72] Inventors **Peter Bruck**  
Encino;  
Nancy Gershman Adin, San Gabriel, both  
of Calif.  
[21] Appl. No. **631,141**  
[22] Filed **Apr. 17, 1967**  
[45] Patented **Oct. 26, 1971**  
[73] Assignee **Bell & Howell Company**  
Chicago, Ill.

[54] **IMPROVED IMAGE INTENSIFICATION FOR  
SENSITIZED FILMS**  
6 Claims, No Drawings

[52] U.S. Cl..... **96/27,**  
96/48, 96/90, 96/89, 96/119, 96/106  
[51] Int. Cl..... **G03c 5/04,**  
G03c 5/24  
[50] Field of Search..... **96/89, 90,**  
106, 101, 48, 27

[56]

**References Cited**

**UNITED STATES PATENTS**

|           |         |                     |         |
|-----------|---------|---------------------|---------|
| 3,486,898 | 12/1969 | Wainer .....        | 96/90   |
| 3,510,300 | 5/1970  | Fatland et al ..... | 96/48   |
| 3,042,517 | 7/1962  | Wainer .....        | 96/90 X |
| 3,095,303 | 6/1963  | Sprague et al ..... | 96/36.3 |
| 3,099,558 | 7/1963  | Levinos .....       | 96/36.3 |
| 3,189,456 | 6/1965  | Hunt .....          | 96/106  |

Primary Examiner—Norman G. Torchin

Assistant Examiner—Richard E. Fichter

Attorney—Robert Berliner

**ABSTRACT:** In a process in which a spectral sensitizer is incorporated in a photosensitive composition to increase its sensitivity to light levels lower than ordinarily useful for inducing a light intensifiable latent image, the improvement wherein the sensitizer has a conjugated system including at least one ring and as a substituent on the ring a group which influences the electron density of the sensitizer to enhance the intensification propensity of the composition.

IMPROVED IMAGE INTENSIFICATION FOR  
SENSITIZED FILMS

## BACKGROUND OF THE INVENTION

## 1. Field of the Invention

The field of art to which the invention pertains includes the field of photographic chemistry, processing and materials, particularly processes involving developing and ancillary operations and compositions therefor, and light-sensitive compositions including those involving light-sensitive dyes and dye formers.

## 2. Description of the Prior Art

Image-intensification methods for increasing film speed to develop-out an image are known to the art. In the field of silver halide photochemistry, several procedures are available for latent image intensification (latensification). Thus, it is known to intensify by means of certain liquid baths, by gaseous treatment or by means of supplemental exposure, or by an assortment of various exposure combinations involving solarization and/or Herschel effects. In the field of organic photochemistry, not involving the use of a silver halide salt to obtain an image, fewer intensification effects have been noted, but even here certain intensifiable systems have been demonstrated. For example, in U.S. Pat. No. 3,095,303 a photosensitive system is described comprising a styryl dye base, (4-(*p*-dimethylaminostyryl)-guinoline), in combination with an organic halogen compound, wherein image-wise exposure causes conversion of the dye base to the quaternary salt, a colored dye, to yield a negative-working image. In that system, without intensification, high levels of exposure are required to obtain an image. However, by means of light intensification, e.g., with red light, moderate levels of imaging light can be used. Such procedures involve color-forming materials, in this case the styryl dye bases, which are themselves intensifiable. Other systems have been described using leuco crystal violet as the color-forming auto-intensifiable material; e.g., in U.S. Pat. No. 3,121,633 brief exposures to heat (or infrared) intensifies an exposed combination of leuco dye base and tribromoacetophenone.

In such systems, the intensifying radiation either has no color-forming effect on those areas of the film which were not previously exposed or else has a lesser effect than on such pre-exposed areas so that the intensification is sufficiently non-fogging to allow the production of a discernible image. Thus, it is known to intensify images obtained in photosensitive material where the photosensitive material itself yields an image that can be intensified. However, there are many photosensitive systems in which the exposed color-forming material does not alone intensify sufficiently to form a useful image, e.g., many silver halide formulations, and many organic systems.

With organic systems, generally two or more organic materials are involved, other than merely dye bases, which react under the influence of actinic light to produce a color. As early as 1921, Murray C. Beebe and his coworkers described numerous organic photographic systems (e.g., U.S. Pat. Nos. 1,574,357; 1,574,358; 1,574,359; 1,575,143; 1,583,519; 1,587,269; 1,587,519; 1,587,270; 1,587,271; 1,587,272; 1,587,273; 1,587,274; 1,604,674; 1,618,505; 1,655,127; 1,658,510; and 1,820,593). Generally, these systems relate to the use of organic halogen compounds (e.g., iodoform and others) in combination with a second material, in which Beebe and subsequent workers have theorized that light effects the release of a radical from the halogen compound which carries out a color-forming reaction with the second material. Subsequent workers such as Eugene Wainer (e.g., U.S. Pat. Nos. 3,042,515; 3,042,516; 3,043,517; 3,042,518; 3,042,519; 3,046,125; and 3,056,673 and Robert Sprague U.S. Pat. No. 3,082,086), as well as a number of other workers since the time of Beebe, have continued the development of various photographic systems involving photo-energized reactions of combinations of halogen-containing compounds and one or more other compound. Other

recent disclosures include British Pat. No. 917,919 and Belgian Pat. No. 596,094. It has also been discovered that incorporation of the above combinations as dispersions in a continuous phase, e.g., gelatin, in which such combinations are substantially insoluble, results in photographic compositions of superior speed, sensitivity and other properties, including, with certain reactants, the ready ability to yield positive-mode pictures, e.g., as described in Belgian Pat. 647,584 and in the above noted applications of Y. Yamada and T. H. Garland.

More recently, it has been found that photosystems as described above and others can be photolatensified by incorporating a material that imparts a photo-latensification propensity to the photosystem. Thus, a sensitizer is incorporated that upon imagewise exposure confers on the composition, in areas of such exposure, increased sensitivity to radiation in a spectral region of lower sensitivity in absence of the sensitizer. The imaged composition is then subjected to such lower sensitivity radiation and the latent image formed upon first exposure is thereby intensified. For example, the photosystem comprising N-vinylcarbazole and carbon tetrabromide, dispersed in gelatin, can yield a positive image under average daylight conditions, and appropriate post-exposure treatment, with an exposure of several seconds. By adding a sensitizer, such as 4-(*p*-dimethylaminostyryl)-quinoline, exposure time can be reduced to one or two seconds to obtain a good positive image. However, if after exposure the composition is blanket exposed to suitable latensifying radiation, in this case red light, good positive images can be obtained with initial exposures of only fractions of a second.

The foregoing and other latensification procedures are described in detail in the above referenced application by Y. Yamada and T. H. Garland entitled "PHOTOGRAPHIC PROCESS." The application notes that the sensitizer imparts sensitivity, upon image-wise exposure, to radiation in a region to which the original material has relatively lower sensitivity, so that upon blanket exposure to such radiation essentially only the imaged areas will be thereby affected. The application further notes that certain sensitizers may impart sensitivity only to radiation in a region to which the original material is highly sensitive, and thus, with such sensitizers latensification is somewhat masked by fogging. In some other cases the imparted sensitivity, although into a relatively nonfogging region, is not of sufficient intensity to effect an entirely satisfactory latensification. Thus some sensitizers are relatively less effective than others.

## SUMMARY OF THE INVENTION

It is now been found that the foregoing, relatively less effective, sensitizers can be improved in their ability to latensify by providing the sensitizer with a molecular group that influences its electron density. In accordance with one aspect of our invention, we provide a means for improving the latensification propensity of a sensitizer by providing it with a substituent that influences its electron density so as to increase such propensity. In another aspect, we provide the composition obtained by combining such improved sensitizer with an image-yielding photosensitive material. In still another aspect of our invention, we provide, as new compounds, substituted dialkylaminostyryl compounds, and vinyl homologs thereof, having the formula



wherein R<sup>1</sup> and R<sup>2</sup> are each independently selected from aromatic and aliphatic groups, n signifies from 1 to a plurality of -CH<sub>2</sub>CH<sub>2</sub>- groups, Y is selected from chlorine, bromine, nitro and methoxy and Z represents atoms selected from C, O and N necessary to complete a fused ring group containing from two to three rings.

## DESCRIPTION OF THE PREFERRED EMBODIMENTS

As noted, improved sensitizers of our invention are materials that upon initial exposure to light sensitize the composition to which they are added to radiation in a region of the spectrum to which the composition otherwise has lower sensitivity. Preferably, the improved sensitizer itself absorbs radiation in a region of the spectrum used for the imaging exposure and, at least in conjunction with the photosensitive composition, responds to such exposure to intensify, extend or shift the sensitivity of the system in or into a region of the spectrum to which the unexposed composition (including the sensitizer) has significantly lower sensitivity. Thus, it is preferred that the substituted sensitizer be a material which imparts selective light absorptivity to the system in which it is incorporated, which absorptivity is shiftable, extensible or, in part, intensifiable as described. In general, it is preferred that the materials have the optical properties of, or be, optical sensitizing dyes or dye bases.

For materials that can be improved by substitution in accordance with our invention, reference can be made to the above-noted Y. Yamada and T. H. Garland applications, particularly the application entitled "PHOTOGRAPHIC PROCESS," and Ser. No. 523,705, now Pat. No. 3,503,745 and reference can also be made to a publication of Brooker and Vittum entitled "A Century of Progress in the Synthesis of Dyes for Photography" in the Journal of Photographic Science, Volume 5, 1957, pp. 71-88, the disclosure of these references being incorporated herein by reference. All of these sensitizers tend to absorb actinic energy and all have exhibited their ability to transmit the absorbed energy by a physical molecular contact or by engagement to other molecules receptive of actinic energy for purposes of modifying the photo-response. Illustrative materials are compounds having a characteristic rhodamine ring structure and nominal substitution at an amino group, such as the rhodamines (i.e., aminophthaleins); materials having simple (unsubstituted) carbon chains interconnecting fused heterocyclic and benzeneoid ring structures, such as pinacyanole and related carbocyanine or cyanine type dyes or dye bases; light absorbers containing heterocyclic rings fused with benzeneoid rings, such as eosin dyes; and light absorbers having a triphenylmethane structure, including leuco forms thereof and compounds having thiazine, alizarine, acridine and anthraquinonoid groups or structures. In general, light absorbers having a styryl substituent such as the styryl and azastyryl dyes and dye bases styryl substituent such as the styryl dye azastyryl dyes and dye bases and vinyl homologs thereof are particularly improved when substituted in accordance with our invention and comprise a particularly preferred group of sensitizers.

As substituents, one can use any electron density influencing group and in a position on the sensitizer that allows the group to influence electron density to increase the photo-latensification propensity of the composition. Thus, both electron-donating and electron-withdrawing groups can be used. Examples of electron-donating groups include:  $-F$ ,  $-Cl$ ,  $-Br$ ,  $-I$ ,  $-OR$ ,

$-O-C(=O)-R$ ,  $-SR$ ,  $-NR_2$ ,  $-NH-C(=O)-R$ ,  $-O-$ ,  $-S-$ ,  $-CR_3$ , and the like. Examples of electron-withdrawing groups include:  $-NO_2$ ,

$-C\equiv N$ ,  $-CHO$ ,  $-C(=O)-R$ ,  $-C(=O)-OR$ ,  $-C(=O)-NR_2$ ,  $-S(=O)-R$ ,  $-CF_3$ ,

and the like.

In the foregoing each R is independently selected from hydrogen, aromatic groups and aliphatic groups. Note that while all of the halogens have been described as electron-

donating groups they actually exhibit both electron-withdrawing and electron-donating properties with the electron-withdrawing effect becoming increasingly more important as one goes down the Periodic Group from fluorine to iodine. Accordingly, the halogens can also be included among electron-withdrawing groups.

In general, it is preferred that the sensitizer have at least one ring as part of a conjugation system, preferably as part of a fused ring group, with the electron density influencing group 10 substituted on the ring. Generally, the position of the substituent depends on whether it is electron-donating or withdrawing. in the case of electron-donating groups it is preferred to add these to a position on the ring ortho or para to a heterocyclic atom or major functional group, or in conjunction with such ortho or para position. in the case of electron-withdrawing atoms or groups, it is preferred to add these to the meta, or conjugatively equivalent, position. However, there are exceptions to these general preferences. As noted, the halogens exhibit both electron-withdrawing and electron-donating properties. Also, some substituents increase the latensification ability of a sensitizer regardless of its position on the ring (this latter effect is particularly notable with electron-withdrawing groups).

Methods of preparing the foregoing sensitizers are well known to the art. Many sensitizers substituted in accordance with our invention are well known as are methods for their preparation. Generally, substitution of the desired electron-influencing group on a precursor to the sensitizer is a convenient 20 method of obtaining the substituted sensitizer. As noted, substituted styryl and azastyryl dyes or dye bases and vinyl homologs thereof are particularly preferred sensitizers in our invention. It is further preferred that the sensitizer have the formula



40 wherein  $R^1$  and  $R^2$  are each independently selected from aromatic and aliphatic groups,  $n$  signifies from 1 to a plurality of 45  $-CH_2-CH-$  groups,  $X$  is an electron density influencing group and  $Z$  represents atoms selected from C, O and N necessary to complete the fused ring group containing from two to three rings. Sensitizers in which  $X$  is halogen, nitro, methoxy, trifluoromethyl, formyl or alkylsulfone are particularly 50 preferred as generally more effective.

The foregoing compounds can be readily prepared by the condensation of an appropriate aromatic aldehyde, e.g., benzaldehyde, cinnamaldehyde, cinnamylidene-acetadehyde, or aldehyde having a larger number of groups, with an appropriately substituted fused ring compound. Examples of suitable fused ring dye precursors include: 4-chloroquinidine; 2-chloropidine, 5-nitroquinidine; 3-methyl-5-nitroisoquinidine; 2-methyl-4-fluoro-1,8-naphthyridine; 2-methyl-5-cyano-1,8-naphthyridine; 2-methyl-4-methoxy-1,7-phenanthroline; 2-methyl-5-formyl-1,7-phenanthroline; 3-methyl-benzo[h]isoquinoline-5-methylsulfone; 2-methyl-4-thiomethyl-5H-pyrido[2,3-d][1,2]oxazine; 2-amino-4-methyl-5H-pyrido[2,3-d][1,2]oxazine; 2-methyl-1,5-pyridine-65 3-[N,N-dimethyl]-carboxamide; N-4-(2-methyl-1,5-pyridinyl-acetamide; 2-methyl-3-acetylpyrido[3,4-b]pyridine; 2-ethyl-4-methylpyrido[3,4-b]pyridine; 2-methyl-3-trifluoromethylpyrido[3,2-b]pyridine; 3-bromo-4-methyl-pyrido[3,2-b]pyridine; 2-methyl-3-iodopyrido[4,3-b]pyridine; and 3-carbomethoxy-4-methylpyrido[4,3-b]pyridine. Examples of aldehyde precursors include: p-dimethylaminobenzaldehyde; o-dimethylaminocinnamaldehyde; m-dimethylaminocinnamylidineacetaldheyde; o-diethylaminobenzaldehyde; m-di-octylaminocinnamaldehyde; p-di-n-propylaminocinnamylidineacetaldheyde; m-di-sec-butyl-aminobenzaldehyde; p-

dimethylaminocinnamaldehyde; and o-dimethylaminocinnamylidineacetaldehyde.

A particularly useful group of sensitizers comprise compounds having the formula



wherein R<sup>1</sup>, R<sup>2</sup>, n and Z are the same as above and Y is selected from chlorine, bromide, nitro and methoxy. Such materials are particularly suited to our invention. Examples include 2-(p-dimethylaminostyryl)-4-chloroquinoline; 2[6-(o-diethylaminophenyl)-1,3,5-hexatrienyl]-4-methoxy-1,7-phenanthroline; 4-[4-(m-di-t-octylaminophenyl)-1,3-butadienyl]-2-nitro-5H-pyrido[2,3-d][1,2]oxazine; 2[6-(p-dimethylaminophenyl)-1,3,5-hexatrienyl]-4-chloroquinoline; 2-(p-dimethylaminostyryl)-4-methoxyquinoline; 4-(p-dimethylaminostyryl)-2-methoxyquinoline; 2-(p-dimethylaminostyryl)-4-trifluoromethylquinoline; 4-(p-dimethylaminostyryl)-2-trifluoromethylquinoline; 4-(o-diethylaminostyryl)-2-bromoquinoline; and 2[4-(p-dimethylaminophenyl)-1,3-butadienyl]-4-chloroquinoline. Derivatives of quinaldine (i.e., 2-methylquinoline) and lepidine (i.e., 4-methylquinoline) are particularly preferred.

With reference to groups designated by the letter "R," it is preferred that when aliphatic they be alkyl, cycloalkyl or aralkyl, and that when aromatic they be aryl or alkaryl. It is further preferred that alkyl be from 1 to about 8 carbon atoms, cycloalkyl be from 5 to about 12 carbon atoms, aryl be from 6 to about 12 carbon atoms, aralkyl be from 7 to about 12 carbon atoms and alkaryl be from 7 to about 12 atoms.

With reference to the letter "n" designating from 1 to a plurality of olefinic groups, n can range from 1 up to any number that is practical; the plurality of compounds thereby represented all possess similar optical properties. It is preferred that n be from 1 to 3 as these compounds are more readily prepared than higher homologs.

The following examples illustrate the preparation of substituted optical sensitizers.

#### EXAMPLE 1

One-tenth mole of each of 4-chloroquinaldine and p-dimethylaminobenzaldehyde and 5ml. of concentrated hydrochloric acid were heated on a hot water bath for 20 hours. A solid mass resulted which was ground under sodium hydroxide solution, extracted into benzene and chromatographed on acidic alumina. Unchanged aldehyde and 4-chloroquinaldine were eluted with benzene and subsequent elution with ether yielded 2-(p-dimethylaminostyryl)-4-chloroquinoline as yellow needles which were recrystallized from methanol as chunky prisms with a melting point of 129-130°C.

#### EXAMPLE 2

One-tenth mole of each of 5-nitroquinaldine and p-dimethylaminobenzaldehyde were condensed using 5ml. of concentrated hydrochloric acid as a catalyst in a manner similar to that of example 1. The product was neutralized with potassium hydroxide, filtered and air dried to yield 2-(p-dimethylaminostyryl)-5-nitroquinoline with a melting point of 170°C.

#### EXAMPLE 3

One-tenth mole of each of 6-dimethylaminoquinaldine and p-dimethylaminobenzaldehyde were refluxed in 50ml. of acetic anhydride for five and one-half hours. The solution was neutralized with excess sodium hydroxide solution and the resultant product was chromatographed on basic alumina with

30

35

40

45

50

55

60

65

70

75

benzene. The original benzene eluate was added to a 50/50 mixture of ligroin and acetone to precipitate 2-(p-dimethylaminostyryl)-6-dimethylaminoquinoline as yellow prisms which were found to have a melting point of 204-207°

6

C.

#### EXAMPLE 4

In a manner similar to that of example 1, one-tenth mole of each of 2-chlorolepidine and p-dimethylaminobenzaldehyde were condensed using 5ml. of concentrated hydrochloric acid as catalyst and chromatographed on alumina to obtain 4-(p-dimethylaminostyryl)-2-chloroquinoline having a melting point of 132-134°C.

In a similar manner, other substituted optical dyes can be prepared from the condensation of an appropriate aldehyde and substituted fused ring group. For example, p-dimethylaminobenzaldehyde can be separately condensed in concentrated hydrochloric acid, as in example 1, with 4-methoxyquinaldine, 2-methoxylepidine, 4-trifluoromethylquinaldine and 2trifluoromethyllepidine to yield, respectively, 2-(p-dimethylaminostyryl)-4-methoxyquinoline, 4-(p-dimethylaminostyryl)-2-methoxyquinoline, 2-(p-dimethylaminostyryl)-4-trifluoromethylquinoline and 4-(p-dimethylaminostyryl)-2-trifluoromethylquinoline.

In general, any photographic system, organic or inorganic, which in its basic form is not uniformly panchromatic but which is capable of having its spectral sensitivity extended, or in part increased, can be improved by the use of a sensitizer of our invention. Such photosensitive systems are described in detail in the above-referenced Yamada and Garland applications. With certain photosystems, a photo-initiator may be desired, e.g., an organic halogen such as carbon tetrabromide, and the use of such materials is also described in the above-noted Yamada and Garland applications. In referring to photographic systems we intend to include not only image-yielding materials which contain color-forming ingredients but also those which yield a color upon subsequent external treatment, e.g., by washing with a coloring agent or by printing with the material or otherwise using it as a master, or by other methods. In referring to the word "image" the term is used to include images which, even in their developed state, are not necessarily discernible to the eye but which are defined by a useful change in physical or chemical properties, such as photographic sensitivity, solubility, wettability, optical turbidity, hardness, surface smoothness, and the like. The image may comprise a desensitization, which may be colorless, of otherwise photosensitive material in light-struck areas so that on still further treatment, color is formed in nonimage areas.

A suitable concentration of our sensitizer depends on the particular photosystem and sensitizer. Many of our sensitizers are capable of forming their own color but this property is not important to the process except insofar as related to an ability to selectively absorb and/or transfer electromagnetic radiation. Thus, a sensitizing amount of the sensitizer is used rather than a color-forming amount, which amounts may be different. In general, about 0.001 to about 100mg. of sensitizer per gram of image-yielding material is satisfactory.

Use of substituted sensitizers of our invention to latensify can be illustrated by the following example.

#### EXAMPLE 5

Test amounts of 2-(p-dimethylaminostyryl)-4-chloroquinoline were prepared as in example 1 and used in a formulation as follows:

|                                                           |          |
|-----------------------------------------------------------|----------|
| 20% Gelatin                                               | 50 ml.   |
| 37% Formalin                                              | 2 drops  |
| 5% Chrome Alum                                            | 5 drops  |
| 1.5% Tergitol 4                                           | 10 drops |
| N-vinylcarbazole                                          | 4.0 g.   |
| Carbon tetrabromide                                       | 3.2 g.   |
| 2-(p-dimethylaminostyryl)-4-chloroquinoline(4-chloro-2SQ) | 3 mg.    |

in ethyl acetate 2 ml.

Baryta paper was coated to about 3 mil wet thickness with the above formulation. Another baryta sheet was coated with a similar formulation but one in which 3mg. of 2-(p-dimethylaminostyryl)-quinoline (2SQ) was substituted for the 4-chloro-2SQ. Test strips of each formulation were exposed for 0.2 and 0.3 seconds to a Kodachrome projection from 34 inches using a 300 Watt Bell & Howell Headliner Projector. One-half of each test strip was covered and the strips were then exposed for 60 seconds to latensifying tungsten light filtered through a Corning CS2-59 red-passing filter (having a cut wavelength of from 6280 to 6370A) at about three feet using the Bell & Howell projector. The coverings were removed and the strips were flooded with a Sylvania "Sun Gun 11" Model SG-55) for one-half second at about 14 inches and then heated by passing through a rotating drum heater at about 70° C. for about ten seconds. Both test strips that were exposed for 0.3 seconds showed an image in the latensified portion and no image in the covered portion; the image obtained with the formulation containing 4-chloro-2SQ was of substantially better contrast. The test strip that was exposed for 0.2 seconds and contained 4-chloro-2SQ showed an image in the latensified portion and not in the covered portion. The test strip that was exposed for 0.2 seconds and contained 2SQ did not show an image in either the latensified or covered portions.

It will be understood that modifications and variations may be effected without departing from the scope of the novel concepts of our invention.

We claim:

1. In a photographic process in which a photosensitive composition is image-wise exposed, an image is formed therein and color is developed in either the image-wise exposed areas or non-image-wise exposed areas of said composition said composition including a photoinitiator component which produce free radicals or ions upon exposure to light of a suitable wavelength, the improvement comprising the steps, prior to complete color development, of:

incorporating in said composition a sensitizing amount of a photographic sensitizing dye or dye base compound which enables an image to be developed in said composition following exposure to actinic radiation normally insufficient to produce said image, said dye or dye base compound being different from other components of said composition and having a conjugated system including at

least one ring and as a substituent on said ring a group which influences the electron density of said dye or dye base compound, whereby said sensitized composition has (1) relatively low or no photosensitivity to light of a first spectral region, (2) high photosensitivity to light of a second spectral region, relative to its photosensitivity to said first spectral region, (3) photosensitivity to light of a third spectral region in portions of said sensitized composition which have been previously exposed to light of said second spectral region, and (4) a coincident range in said first and third spectral regions; imagewise exposing said sensitized composition with light of said second spectral region sufficient to radiatively modify said composition to constitute a latent image; and blanket exposing said image-wise exposed composition with light of said coincident range to further radiatively modify those portions of the composition constituting said latent image.

2. The process of claim 1 wherein the sensitizing compound is of a series selected from the rhodamine, pinacyanole, cyanine, eosin, triphenylmethane, thiazine, anthraquinonoid, acridine and styryl dye and dye base series.

3. The process of claim 1 wherein the sensitizing compound has the formula



wherein R<sup>1</sup> and R<sup>2</sup> are each independently selected from aromatic and aliphatic groups, n signifies from 1 to a plurality of -CH<sub>2</sub>CH- groups, X is an electron density influencing group and Z represents atoms selected from C, O and N necessary to complete a fused ring group containing from 2 to 3 rings.

4. The process of claim 3 wherein X is selected from halogen, nitro, methoxy, trifluoromethyl, formyl and alkylsulfone.

5. The process of claim 3 wherein the sensitizer is a dialkylamino-styrylquinoline.

6. The process of claim 5 wherein X is selected from halogen, nitro, methoxy, trifluoromethyl, formyl and alkylsulfone.

UNITED STATES PATENT OFFICE  
CERTIFICATE OF CORRECTION

Patent No. 3,615,430 Dated October 26, 1971

Inventor(s) Peter Bruck, et al

It is certified that error appears in the above-identified patent and that said Letters Patent are hereby corrected as shown below:

Column 1, line 3, before "BACKGROUND OF THE INVENTION", insert the following material: -- CROSS-REFERENCE TO RELATED APPLICATIONS Related disclosures are contained in the following applications by Y. Yamada and T.H. Garland: "PHOTOGRAPHIC PROCESS," Serial No. 631,502, filed concurrently herewith; "DYE SENSITIZATION," Serial No. 523,705, filed January 28, 1966, now U.S. Patent No. 3,503,745; "PRODUCTION AND USE OF PHOTOSENSITIVE COMPOSITIONS AND FILMS," Serial No. 481,759, filed August 23, 1965, now U.S. Patent No. 3,476,562; and "DYE SENSITIZATION OF PHOTOSENSITIVE MATERIALS," Serial No. 352,625, filed March 17, 1964, now abandoned. -- ; line 27, "guinoline" should read -- quinoline -- . Column 2, line 72, " -CH CH-" should read --- -CH=CH- -- . Column 4, line 12, "in" should read -- In -- ; line 15, "in" should read -- In -- ; line 38, change



line 45, change " -CH CH-" to read --- -CH=CH- -- ; line 54, after "of" insert --- -CH=CH- -- ; line 65, after "1,5-pyridinyl" insert -- ) -- .

UNITED STATES PATENT OFFICE  
CERTIFICATE OF CORRECTION

Patent No. 3,615,430 Dated October 26, 1971

Inventor(s) Peter Bruck, et al -2-

It is certified that error appears in the above-identified patent and that said Letters Patent are hereby corrected as shown below:

Column 5, line 8, change "



Y

line 14, after "chlorine" change "bromide" to read -- bromine -- ;  
line 36, after "12", second occurrence, add -- carbon -- .  
Column 7, line 16, before "Model" add -- ( -- ; line 38,  
"produce" should read -- produces -- . Column 8, line 35, change  
"--CH CH--" to read -- -CH=CH- -- .

Signed and sealed this 14th day of November 1972.

(SEAL)  
Attest:

EDWARD M. FLETCHER, JR.  
Attesting Officer

ROBERT GOTTSCHALK  
Commissioner of Patents